



US005863455A

**United States Patent** [19]**Segal**[11] **Patent Number:** **5,863,455**[45] **Date of Patent:** **Jan. 26, 1999**[54] **COLLOIDAL INSULATING AND COOLING FLUID**[75] Inventor: **Vladimir Segal**, Livingston, N.J.[73] Assignee: **ABB Power T&D Company Inc.**, Raleigh, N.C.[21] Appl. No.: **892,054**[22] Filed: **Jul. 14, 1997**[51] **Int. Cl.** **6** **H01F 1/44; H05K 5/00; F25B 21/00; B01J 13/00**[52] **U.S. Cl.** **252/62.52; 252/62.54; 252/62.51 R; 252/308; 252/309; 252/311; 252/313.1; 62/3.1; 361/699; 361/698**[58] **Field of Search** **252/62.52, 62.54, 252/62.51 R, 308, 309, 311, 313.1; 62/3.1; 361/699, 698**[56] **References Cited**

## U.S. PATENT DOCUMENTS

|           |         |                |           |
|-----------|---------|----------------|-----------|
| 3,215,572 | 11/1965 | Papell         | 149/2     |
| 3,301,790 | 1/1967  | Fitch et al.   | 252/308   |
| 3,635,819 | 1/1972  | Kaiser         | 252/62.52 |
| 3,843,540 | 10/1974 | Reimers et al. | 252/62.52 |
| 3,917,538 | 11/1975 | Rosenweig      | 252/62.51 |
| 4,094,804 | 6/1978  | Shimoizaka     | 252/62.52 |
| 4,356,098 | 10/1982 | Chagnon        | 252/62.51 |
| 4,506,895 | 3/1985  | Raj            | 277/1     |
| 4,523,967 | 6/1985  | Cartwright     | 149/2     |

|           |         |                |           |
|-----------|---------|----------------|-----------|
| 4,732,706 | 3/1988  | Borduz et al.  | 252/510   |
| 4,992,190 | 2/1991  | Shtarkman      | 252/62.52 |
| 5,188,764 | 2/1993  | Shimizu et al. | 252/308   |
| 5,382,373 | 1/1995  | Carlson et al. | 252/62.55 |
| 5,462,685 | 10/1995 | Raj et al.     | 252/62.52 |

## OTHER PUBLICATIONS

Publication entitled, "Transformation" (for employees of the ABB Power Transformer Division): Issue 3, Jan. 29, 1990; Issue 7, Mar. 26, 1990, Issue 11, May 21, 1990; Issue 12, Jun. 4, 1990, Issue 13, Jun. 13, 1990; Issue 14, Jul. 2, 1990, Issue 15, Jul. 16, 1990; Issue 24, Nov. 19, 1990, Issue 25, Dec. 3, 1990; Issue 32, Mar. 11, 1991, Issue 34, Apr. 8, 1991. B. Berkovsky and V. Bashtovoy, Eds., *Magnetic Fluids and Applications Handbook*, Begall Publishing House, New York, New York (1996), no month.

Primary Examiner—Melissa Bonner  
Attorney, Agent, or Firm—Woodcock Washburn Kurtz Mackiewicz & Norris LLP

## [57]

## ABSTRACT

Colloidal fluids having improved insulating and/or cooling properties. Embodiments of the invention involve colloidal fluids which comprise a carrier liquid and a dispersed phase of non-metallic particles, wherein the colloidal fluid has a saturation magnetization of less than about 50 Gauss. The compositions may be employed to insulate and/or cool electromagnetic devices, including high power devices, such as power transformers.

25 Claims, 1 Drawing Sheet





**Fig. 1**

## COLLOIDAL INSULATING AND COOLING FLUID

### FIELD OF THE INVENTION

The present invention relates to novel colloidal fluids. More particularly, the present invention relates to novel colloidal fluids and their use for insulating and/or cooling electromagnetic devices.

### BACKGROUND OF THE INVENTION

Liquid insulation in an electromagnetic device, such as a power transformer, is subject to different types of voltages: AC voltages having a wide range of amplitudes and frequencies, and impulse (essentially, short-lived DC) voltages of even higher amplitude. The ability of liquid insulation to withstand the stresses imposed by electric fields of a particular voltage is often the most important property of such an insulation. This determines whether a particular liquid can be used as an insulation in a transformer (or any other electromagnetic device where high voltage is employed) of a given voltage rating. The selection of an insulation is important in that it can determine the design of all of the main elements of the device.

Typically, the highest voltage stressing the liquid insulation is the impulse (lightning) voltage. When the volume of liquid insulation is subjected to a critical dielectric stress produced by rising to its peak value impulse voltage, an insulation breakdown may occur.

To maximize the efficiency of electrical energy transmission and distribution, it is often necessary to utilize high current densities and high AC voltages inside the electromagnetic device. High currents lead to increased heat generation, while high voltage increases the level of electric stress applied to the insulation components of an electromagnetic device. Increased heat generation limits the maximum current which can be safely carried by the conductive elements of an electromagnetic device, and also increases the costs associated with the transmission, distribution, and final use of electrical energy due to the increased need for conductive materials. This also results in an overall increase in the weight and size of a given electromagnetic device. High electric stress also limits the voltage drop per unit of space inside an electromagnetic device, thereby leading to increased costs associated with the transfer of energy from generation point to the final user. Moreover, to compensate for higher stress, it is often necessary to increase the space between winding turns filled with insulation liquid, such as transformer oil, thereby further increasing transformer dimensions and cost.

Since electric current generates both heat and electric stress, it is important that the electric insulation performs two different functions continuously: (a) prevents current flow between different conductive components having different voltages; and (b) transfers heat from the windings and magnetic core to the outer walls of the device to be cooled. The dielectric properties of the liquid insulation are the most critical ones, for they are responsible for the functioning of a high voltage electromagnetic device, and dielectric strength of an insulation liquid cannot be compromised. As a result, practically all prior art liquid insulation systems have substantially high dielectric strength, low electric conductivity and high levels of purity; it is believed that this latter property is necessary for desirable dielectric strength. However, liquid insulation systems of the prior art also possess low heat conductivity, which prevents efficient heat transfer via conduction. Instead, electromagnetic devices

generally employ Archimedes convection which results from the expansion of liquid insulation, e.g., transformer oil, upon heating to elevated temperatures so an Archimedes force develops which lifts the hot (and less dense) oil up and pushes the cold (more dense) oil down. Thus, thermal convection is established and heat transfer becomes possible from the windings to the outer wall of an electromagnetic device. This type of heat transfer, however, has relatively low efficiency and requires that there be provided special paths (ducts) inside the windings and the magnetic core so that the oil can flow through the hottest inner sections of the parts of the device which generate heat. Relying on heat transfer through the rather inefficient mechanism of Archimedes convection leads to an increase in the size of the device as well as an increase in cost by lowering the amount of conductive or magnetic material per unit volume. Moreover, even if the necessary precautions have been taken to ensure heat transfer, so-called hot spots can develop inside the windings/magnetic core assembly which further limits the voltage and current.

Prior art liquid insulation systems perform their functions within a limited range of current, voltage, and environmental conditions which define the power rating of an electromagnetic device. There is a need to expand these limits so that high power, i.e., higher voltage or current, can be transmitted via the device without compromising its safety and reliability, or so that the same power can be transmitted but with a smaller and less costly device. The present invention is directed to this, as well as other important ends.

### SUMMARY OF THE INVENTION

The present invention relates, in part, to colloidal fluids. Specifically, in one embodiment, the invention relates to a stable, colloidal fluid comprising (a) about 99.99 to about 98% by volume of a carrier liquid, and (b) from about 0.01 to about 2% by volume of non-metallic particles, wherein the colloidal fluid has a saturation magnetization of less than about 50 Gauss.

Another embodiment of the invention relates to a stable, colloidal fluid which comprises (a) a carrier liquid, and (b) non-metallic particles, wherein the colloidal fluid has a saturation magnetization of less than about 50 Gauss.

Still another embodiment of the invention relates to a method for preparing a colloidal fluid having a saturation magnetization of less than about 50 Gauss. The method comprises (a) providing a carrier liquid, and (b) combining non-metallic particles with the carrier liquid.

Yet another embodiment of the invention relates to an electromagnetic device. The device comprises (a) means for producing an electromagnetic field and heat, and (b) a stable, colloidal fluid which is in contact with the device. The colloidal fluid comprises (i) a carrier liquid, and (ii) non-metallic particles, wherein the colloidal fluid has a saturation magnetization of less than about 50 Gauss.

Still another embodiment of the invention relates to a method of insulating and cooling an electromagnetic device which produces an external magnetic field and heat. The method comprises contacting the device with a stable, colloidal fluid comprising (a) a carrier liquid, and (b) non-metallic particles. The colloidal fluid has a saturation magnetization of from greater than 0 to less than about 50 Gauss.

These and other aspects of the invention will become more apparent from the present description and claims.

### BRIEF DESCRIPTION OF THE DRAWINGS

For the purpose of illustrating embodiments of the invention, there is shown in the drawings forms which are

presently preferred. It should be understood, however, that this invention is not limited to the precise arrangements and instrumentalities shown.

FIG. 1 is a schematic representation of a transformer including a system for cooling the transformer in accordance with an embodiment of the present invention.

#### DETAILED DESCRIPTION OF THE INVENTION

The present invention is directed, in part, to novel colloidal fluids for use, for example, in connection with electromagnetic devices. The term "colloid", as used herein, refers to a state of subdivision of matter which may comprise single large molecules, or aggregations of smaller molecules. Within the colloid, particles of ultramicroscopic size, which are often referred to as the dispersed phase, are generally surrounded by different matter, which is often referred to as the carrier liquid, dispersion medium or external phase. The size of the particles included in the colloids of the present invention may vary depending, for example, on the particles employed, the particular application, and the like. Generally speaking, the particle size preferably ranges from about 1 to about 100 nanometers, and all combinations and subcombinations of ranges therein. Thus, the colloids of the present invention may generally be referred to as "nanofluids". In certain embodiments of the present invention, the particles in the colloids may be magnetic. The term "magnetic", as used herein, refers to the property of substances which, under certain conditions, attract or repel each other. An example of a colloid which contains magnetic particles is a "ferrofluid". The ferrofluids described herein may respond to an applied magnetic field as if the fluid itself possessed magnetic characteristics. In certain other preferred embodiments of the present invention, the colloids contain particles which are non-magnetic. The term "non-magnetic", as used herein, refers to the substantial (including complete) lack of magnetic properties.

The colloids of the present invention preferably address the three fundamental problems described above which may limit the power distributed per unit of the device volume (or weight). Specifically, the present colloids are preferably characterized by one or more of the following properties: (a) higher partial discharge voltage which allows for smaller distances between conductive elements of the device in use by increasing the limits in short term AC fluctuations, (b) increased impulse breakdown strength, so that the transformer can be designed with smaller spacings between the charged parts and with improved reliability under high voltage impulse surges, and (c) increased heat transfer capacity proportional to the magnetic field strength, so that heat is efficiently transferred from inside the windings where the magnetic field is the strongest and where efficient heat exchange is most critical.

Generally speaking, the novel colloids of the present invention may be prepared, for example, by combining particles with a carrier fluid. In a preferred method, the colloids may be prepared by combining colloids having a relatively high concentration of particles with a conventional liquid insulation, such as a conventional transformer oil, to provide nanofluids as described herein. Additional methods for preparing the colloids are discussed more fully herein-after. In preferred embodiments of the present invention, the nanofluids may possess dielectric properties. These dielectric nanofluids may be substantially non-magnetic, or they may possess magnetoactive (magnetic) properties. Exem-

plary among the dielectric nanofluids of the present invention are ferrofluids. The nanofluids described herein may be formulated to obtain the desired properties depending, for example, on the particular application. For example, the nanofluids may be prepared primarily to enhance the insulation dielectric strength. Increasing the volume concentration of the particles may provide a corresponding increase in the saturation magnetization, resulting in an increase in both the insulation dielectric strength and the heat transfer performance of the nanofluid. The colloids may also be formulated to primarily provide desirable heat transfer.

The effect of ferrofluid magnetization saturation and its electric Resistivity (which are determined by the volume percentage of magnetic particles, their average size and its frequency distribution, as well as some ferrofluid manufacturing specifics) on the magnetoactive liquid dielectric strength at AC and DC voltage conditions and on its cooling capacity have been tested in the laboratory and on commercial transformers. The novel colloidal insulation fluids have been developed in such a way that the partial discharge (PD) inception voltage, heat transfer capacity, and impulse breakdown voltage all correlate with two parameters easy to measure after the magnetoactive colloidal liquid is prepared: the magnetization saturation ( $M_s$ ) which, for the applications described and claimed herein, may be about zero (for non-magnetic colloids), or may vary from about 0.5 to about 50 Gs, and electric Resistivity (R) which may vary from about  $10^9$  to more than about  $10^{13}$  Ohm-cm. The actual values of these two parameters depend on a particular combination of insulation properties and cooling capacity needed for a given transformer.

Thus, the colloids of the present invention may possess highly advantageous electrical resistivities, and are therefore especially useful as insulating fluids for electromagnetic devices, including transformer devices. In particular, the colloids of the present invention may provide substantial increases in the minimum (positive) values for impulse breakdown voltage, as compared to the minimum (positive) impulse breakdown values associated with many prior art insulating fluids. In preferred embodiments, the present colloids provide an increase in the positive value of impulse breakdown voltage of at least about 10%, with an increase of more than about 10% being more preferred, including, for example, about 15%. Even more preferably, the present colloids provide an increase in the positive value of impulse breakdown voltage of greater than about 15%, for example, about 20%, with an increase of more than 20% being still more preferred, including, for example, about 25%. Yet more preferably, the present colloids provide an increase in the positive value of impulse breakdown voltage of greater than about 25%, for example, about 30%, with an increase of more than 30% being even more preferred, including, for example, about 35%. Still more preferably, the present colloids provide an increase in the positive value of impulse breakdown voltage of greater than about 35%, for example, about 40%, with an increase of more than 40% being still more preferred, including, for example, about 45%. Yet more preferably, the present colloids provide an increase in the positive value of impulse breakdown voltage of greater than about 45%, for example, about 50%, with an increase of more than 50% being still more preferred.

In addition to the aforementioned desirable insulating properties, embodiments of the present invention provide colloids which may possess highly advantageous heat transfer properties. Accordingly, colloids of the present invention may also be utilized, for example, as cooling fluids to cool electromagnetic devices, including high power transformers,

which operate at elevated temperatures. As known to the skilled artisan, high power transformers typically operate at temperatures of from about 70° C. to about 90° C., and typically have maximum operating temperatures of about 110° C., with temperatures of up to about 130° C. in so-called hot spots. The temperature increase observed when colloidal insulating fluids of the present invention are utilized as cooling fluids may be substantially less than that observed with many prior art insulating and/or cooling fluids. In preferred embodiments, the temperature rise with colloids of the present invention is preferably reduced by at least about 1%, with a reduction in temperature rise of more than 1% being more preferred, including, for example, about 5%. Even more preferably, the temperature rise with colloids of the present invention is preferably reduced by more than about 5%, including, for example, about 10%, with an increase of more than 10% being still more preferred, including, for example, about 15%.

While not intending to be bound by any theory or theories of operation, it is believed that the desirable cooling properties which are achieved with embodiments of the present invention may be due, at least in part, to an advantageous use of magnetic properties. In this connection, and as discussed more fully hereinafter, the present colloids desirably possess a saturation magnetization of up to about 50 Gauss, (preferably less than about 50 Gauss and, in certain preferred embodiments, from greater than 0 to less than about 50 Gauss). Thus, in the case, for example, of colloids containing magnetic particles, magnetic field gradients which may be formed by electromagnetic devices may attract and draw the colloids towards regions of the device where the magnetic field is strongest such as, for example, the windings. This advantageously enhances the convection cycle which is now driven by two forces: magnetic forces and gravitational forces. However, in certain transformer designs including, for example, transformer designs having pancake windings, the magnetic force produces mainly horizontal convection which is perpendicular to the Archimedes component and which may undesirably interfere with the Archimedes flow of the cooling fluid. This horizontal convection may be reduced by limiting the magnetization saturation of the colloidal fluids. Thus, the magnetization saturation for the colloids of the present invention is desirably selected so as to provide advantageous radial or angular convection inside the coil/core assembly and thereby provide improved cooling effects such as, for example, by preventing the formation of undesirable hot spots. At the same time, in regions outside the coil/core assembly, where magnetic fields decrease sharply, the Archimedes convection may prevail, thereby preserving the trajectory of normal (i.e., vertical) liquid circulation.

The colloids of the present invention are preferably highly stable. The term "stable", as used herein, means that the present colloids are substantially or completely resistant to decomposition, including, for example, chemical degradation of the dispersed and/or carrier phase, as well as phase separation of the dispersed and carrier phases, when exposed to varying temperature conditions, including elevated temperatures which may be associated with the operation of electromagnetic devices, such as power transformers, preferably for extended periods of time. Thus, the present colloids are particularly suitable for use, for example, as insulating fluids for electromagnetic devices, including power transformers, which may have extremely long life spans. In preferred form, the colloids of the present invention preferably possess electrical resistivities of at least about  $10^9$  ohm·cm, with electrical resistivities of greater

than about  $10^9$  ohm·cm being more preferred. Even more preferably, the colloids of the present invention possess electrical resistivities of from about  $10^9$  ohm·cm to more than about  $10^{13}$  ohm·cm. As discussed above, the present colloids also possess highly beneficial heat transfer properties. Accordingly, the colloids described herein may be advantageously employed as cooling agents for electromagnetic devices, including electromagnetic devices which operate at high power levels and which may produce significantly elevated operating temperatures, such as power transformers.

A wide variety of materials may be employed in the present colloids, for example, as the dispersed and/or carrier phases. The particular materials which are utilized may vary and depends, for example, on the desired levels of magnetization, cooling properties, electrical resistivity, and the like, as well as the desired application. In preferred form, the dispersed and carrier phases are selected so that the colloids of the present invention have a saturation magnetization ( $M_s$ ) of no greater than about 50 Gauss and preferably, less than about 50 Gauss including, for example, from about 0 to less than about 50 Gauss, and all combinations and subcombinations of ranges therein. In the case of colloids prepared from non-magnetic particles, the colloids may have a saturation magnetization of about 0. In the case of colloids prepared from particles having magnetic properties, the colloids may have a saturation magnetization of from greater than 0 to less than about 50 Gauss. It has been observed that especially advantageous cooling effects may be observed with colloids having a saturation magnetization of from about 0.5 to less than about 50 Gauss, with optimum cooling being observed with saturation magnetizations of from about 20 to about 40 Gauss. Particularly advantageous dielectric strengths are observed when the colloids of the present invention possess a saturation magnetization of from about 0.1 to about 5 Gauss, with optimum dielectric strengths being observed with saturation magnetizations of from about 0.5 to about 2 Gauss. For both desirable cooling and dielectric properties, the colloids of the present invention preferably have saturation magnetizations of from about 1 to about 20 Gauss, with about 5 to about 20 Gauss providing optimum combined properties.

In accordance with preferred embodiments of the present invention, the carrier phase is preferably a liquid which itself is stable, and which provides a desirable and stable environment for the dispersed phase. It is also preferred that the carrier phase possess a low dielectric constant, preferably less than about 3. It is also preferred that the carrier liquid possess a high electrical resistivity level which may enhance the electrical resistivity of the present colloids, as discussed above. The viscosity of the carrier phase may be selected, as desired, to provide desirable stability of the present colloids, as well as advantageous convection cooling, as described herein.

In preferred embodiments, the carrier phase employed in the present colloids is an oil. Exemplary oils include, for example, many of the oils which are currently employed as cooling fluids in high-power transformers. Thus, exemplary oils include, for example, various forms of petroleum, including those of high molecular weight, synthetic hydrocarbons, and silicones. Oils which are particularly suitable for use as the carrier phase in the present colloids are transformer grade mineral oils which are sold under the trade name UNIVOLT™, commercially available from Exxon Corporation (St. Paul, Minn.). Other materials which may be suitable for use as the carrier phase in the colloids described herein would be readily apparent to one of ordinary skill in the art, once armed with the present disclosure.

As noted above, the present colloidal fluids further preferably comprise a dispersed phase, preferably in the form of particles. As with the carrier phase discussed above, a wide variety of materials may be employed as the dispersed phase in the colloids described herein. In preferred embodiments, the dispersed phase is derived from nonmetallic materials. Specifically, it has been observed that improved AC breakdown strengths may be provided when the dispersed phase comprises a non-metallic material. The term "non-metallic", as used herein, refers to materials which may be substantially or completely devoid of metallic properties and/or characteristics. Exemplary non-metallic materials which may be employed as the dispersed phase include, for example, organic materials (such as, for example, polymeric materials), inorganic materials (such as, for example, aerosil), and certain elements, such as elemental carbon. Preferred among these exemplary non-metallic materials are inorganic materials, with metal oxides being particularly preferred among the inorganic materials.

In accordance with certain preferred embodiments of the present invention, the dispersed phase is derived from materials which are magnetic (that is, materials which have an intrinsic magnetic dipole moment), with materials that are both magnetic and non-metallic being preferred. This is because it has been found that both improved AC breakdown strengths and advantageous cooling properties may be obtained when the dispersed phase is both non-metallic and magnetic. It is also preferred that the dispersed phase comprise materials having a Curie temperature of greater than about 200° C. In particularly preferred embodiments, the dispersed phase comprises a magnetic inorganic material, with magnetic metal oxides being yet more preferred. Preferred among these metal oxides are, for example, oxides of iron (such as, for example,  $FeO$ ,  $Fe_2O_3$  and  $Fe_3O_4$ ), zinc (such as, for example  $ZnO$ ), cobalt (such as, for example,  $CoO$ ), manganese (such as, for example,  $MnO$ ,  $Mn_3O_4$  and  $Mn_2O_3$ ), titanium (such as, for example,  $TiO_2$  and  $Ti_2O_3$ ), copper (such as, for example,  $Cu_2O$ ), nickel (such as, for example,  $NiO$  and  $Ni_2O_3$ ), and chromium (such as, for example,  $Cr_2O_3$ ). Preferred also are mixed metal oxides including, for example, oxides of iron and cobalt (such as, for example,  $Fe_2CoO_4$ ), iron, manganese and zinc (such as, for example,  $Mn_xZn_{(1-x)}Fe_2O_4$ , where  $x$  may range from about 0.4 to about 0.8), and iron, cobalt and zinc (such as, for example,  $Co_xZn_{(1-x)}Fe_2O_4$ , where  $x$  may range from about 0.2 to about 0.6). Particularly preferred among the metal oxides are iron oxides. Also in preferred form, the oxides employed have reasonably high magnetization levels which are also substantially dependent on temperature. Viewed from this standpoint,  $Mn_xZn_{(1-x)}$  oxides and iron oxides are most preferred, wherein  $Mn_xZn_{(1-x)}$  oxides are particularly suitable for use under the most demanding conditions (such as, for example, in traction transformers), and iron oxides are particularly suitable for use in conventional distribution and power transformers.

In certain other preferred embodiments of the invention, the dispersed phase may be derived from materials which are non-magnetic. Preferred non-magnetic materials include, for example, organic materials, such as a polymeric material and non-organic aerosils. Preferred among the polymeric materials are fluorinated polymers, including, for example, poly(tetrafluoroethylene), which is commercially available from the DuPont Chemical Co. (Wilmington, Del.) as TEFLON™.

Other materials which may be suitable for use as the dispersed phase in the colloids described herein would be readily apparent to one of ordinary skill in the art, once armed with the present disclosure.

The material which may be utilized as the dispersed phase in the colloids of the present invention is preferably in the form of particles. The size of the particles which are dispersed in the colloid may vary and depends, for example, on the particular dispersed and carrier phases utilized, and the desired application. It is preferred, however, that the size of the particles be selected from among a preferred particle size range. In this connection, it has been found that particle size may affect the cooling and electrical resistivity properties of the colloid. For example, depending on the chemical components of the particles, the use of smaller particles may result in colloids having lower electric resistivity properties which, in use, may result in undesirably high dielectric losses. Conversely, the use of larger particles may, depending on the chemical components of the particles, result in colloids which have poor stability properties, particularly at elevated temperatures. As noted above, preferred particle sizes range from about 1 to about 100 nanometers (nm), and all combinations and subcombinations of ranges therein. More preferably, the average particle size may range from about 5 nm up to about 20 nm, with an average particle size of greater than about 5 nm to less than about 20 nm being even more preferred, including, for example, about 15 nm. Still more preferably, the average particle size may be at least about 7 nm, with about 90% of the particles having a particle size of greater than about 7 nm being particularly preferred.

The concentration of the dispersed phase in the colloids of the present invention liquid may vary and depends, for example, on the particular dispersed and carrier phases utilized, the desired application of the colloid, and the like. If desired, the colloid may be formed initially with the dispersed phase being present in higher concentrations. These concentrated colloids may then be diluted, for example, to achieve a preferred concentration, as discussed more fully hereinafter. In this manner, the colloids of the present invention may provide beneficial versatility, since concentrations may be obtained by the end-user, as desired, depending on the particular application. In this connection, it is contemplated that the dilution may be conducted, for example, at the site of the intended use, such as the manufacturing and/or utility site of a power transformer. The initial preparation of colloids in concentrated form may serve to reduce the volume of the colloid which needs to be shipped to the desired site. This may facilitate transportation of the colloid, for example, by reducing the necessity and/or frequency of shipments of colloid to the site, which may provide significant cost savings.

Broadly speaking, the dispersed phase may be included in the present colloids in a concentration which preferably ranges from greater than about 0% by volume, such as, for example, about 0.01% by volume, up to about 2% by volume, and all combinations and subcombinations of ranges therein. In connection with colloids prepared from dispersed phases which are composed of non-magnetic particles, the concentration of the dispersed phase is preferably from about 0.01% by volume to about 0.5% by volume, with a concentration of from about 0.05% to about 0.3% by volume being more preferred. In connection with colloids prepared from dispersed phases which are composed of magnetic particles, the concentration of the dispersed phase is preferably from about 0.01% by volume to less than 2% by volume, with concentrations of from about 0.02% to about 1% by volume being more preferred.

As would be apparent to one of ordinary skill in the art, once armed with the present disclosure, the amount of carrier phase employed in the colloids described herein may

vary and depends, for example, on the concentration of dispersed phase employed, as discussed above. Thus, generally speaking, the amount of carrier liquid may preferably range from about 99.99% by volume to less than about 98% by volume, including all combinations and subcombinations of ranges therein. In connection with colloids prepared from dispersed phases which are composed of non-magnetic particles, the carrier liquid is preferably present in an amount from about 99.99% by volume to about 99.5% by volume, with a concentration of from about 99.95% to about 99.7% by volume being more preferred. In connection with colloids prepared from dispersed phases which are composed of magnetic particles, the carrier phase is preferably present in an amount of from about 99.99% by volume to greater than about 99.8% by volume, with concentrations of from about 99.98% to about 99% by volume being more preferred.

In addition to the dispersed phase and carrier phase discussed above, the colloids of the present invention may further optionally comprise additional additive materials, including, for example, stabilizing materials, such as, for example, surfactants, dispersants, thickening agents, viscosity modifying agents, antioxidants, and the like. Such materials may be employed, for example, to enhance the stability of the colloids by minimizing or substantially (including completely) preventing phase separation, agglomeration of the dispersed phase, and the like. In preferred embodiments, the optional additive material comprises a surfactant. Preferably, the surfactant contacts or substantially (including completely) coats the particles in the colloid. In the case of particles which are non-magnetic, the particles may be silanized.

A wide variety of surfactants are may be employed in the present colloids. The surfactant may be anionic, cationic or non-ionic, depending, for example, on the particular dispersed and carrier phases employed, and the desired application. Exemplary anionic surfactants include, for example, long-chain (fatty) compounds which contain carboxy groups, succinate groups, phosphate groups, or sulfonate groups. Exemplary cationic surfactants include, for example, long-chain compounds which contain protonated or quaternary ammonium groups. Exemplary non-ionic surfactants include, for example, alcohols and polyoxyalkylene polymers. Other surfactants, in addition to those exemplified above, as well as other optional additive materials suitable for use in the present colloids, would be readily apparent to one of ordinary skill in the art, once armed with the present disclosure.

The concentration of optional additive materials which may be employed in the present colloids may vary and depends, for example, on the particular additive material,

dispersed phase and/or carrier phase employed. Preferably, the additional additive material may be employed in a concentration which enhances desirable characteristics of the colloids, such as, for example, stability, cooling, 5 antioxidant, and/or insulating properties. In preferred embodiments, the optional additive material may be employed in a concentration of from about 0.02% by volume to about 1% by volume, and all combinations and subcombinations of ranges therein.

10 The colloids of the present invention may be prepared using techniques which would be apparent to the skilled artisan, once placed in possession of the present disclosure. For example, colloidal dispersions of particles may be prepared by utilizing methods such as, for example, grinding coarse particles, such as by ball-milling, in the presence of a liquid carrier. The particles resulting from the grinding process may, if desired, be removed from the carrier and then redispersed in a second carrier. Removal of the particles may involve, for example, flocculation. Methods for preparing colloids, including ferrofluids, which may be employed to prepare the colloids of the present invention, are described, for example, in Papell, U.S. Pat. No. 3,215,572, Rosenswieg, U.S. Pat. No. 3,917,538, and *Magnetic Fluids and Applications Handbook*, B. Berkovsky, V. Bashtovoy, 15 Eds., Begall Publishing House, New York, N.Y. (1996), the disclosures of which are hereby incorporated herein by reference, in their entirities.

## EXAMPLES

30 The invention is further described in the following examples. The examples are actual examples and are for illustrative purposes only, and are not to be construed as limiting the appended claims.

### Example 1

35 This example includes a description of experiments which were conducted to evaluate the effect on stability, dielectric strength and dissipation factor of varying concentrations of particles in a transformer oil. The results of these experiments are tabulated in the following Table 1. The compositions studied in these experiments were formulated from UNIVOLT™ 60 oil, which is a transformer grade mineral oil 40 commercially available from Exxon Corporation (St. Paul, Minn.), iron oxide ( $Fe_3O_4$ ) particles as magnetic particles, TEFLO™ particles as non-magnetic particles, and oleic acid as surfactant. The testing methods employed in this 45 example were conducted according to ASTM standards. Impulse breakdown voltage was evaluated according to ASTM D-3300.

TABLE 1

| Particle | Characteristic Measured |               |        |                          |                 |                    |            |               |              |          |
|----------|-------------------------|---------------|--------|--------------------------|-----------------|--------------------|------------|---------------|--------------|----------|
|          | Conc.                   | Ms            | AC     | Dielectric Strength (KV) |                 | Dissipation Factor |            | Loss Increase | Stability    |          |
|          |                         |               |        | Impulse Breakdown        | (tan $\delta$ ) | at 25° C.          | at 100° C. |               |              |          |
| Example  | (Volume %)              | Particle Type | Gauss) | Breakdown                | Positive        | Negative           | at 25° C.  | at 100° C.    | (% of Total) |          |
| 1A       | 0                       | —             | 0      | 55                       | 78              | 151                | 0.005      | 0.04          | 0            | —        |
| 1B       | 5                       | magnetic      | 250    | 46                       | 85              | 135                | >1000      | >1000         | 25           | stable   |
| 1C       | 5                       | non-magnetic  | 0      | 52                       | n/a             | n/a                | n/a        | n/a           | n/a          | unstable |
| 1D       | 2                       | magnetic      | 100    | 47                       | 89              | 120                | 150        | >1000         | 8            | stable   |
| 1E       | 2                       | non-magnetic  | 0      | 53                       | 95              | 140                | 1.5        | 6             | n/a          | unstable |
| 1F       | 1                       | magnetic      | 50     | 49                       | 105             | 110                | 12         | 95            | 5            | stable   |
| 1G       | 1                       | non-magnetic  | 0      | 55                       | 110             | 120                | 0.6        | 3.5           | 0.2          | stable   |

TABLE 1-continued

| Particle | Conc.      | Ms            | Characteristic Measured  |           |           |                    |          |                 |           |            |
|----------|------------|---------------|--------------------------|-----------|-----------|--------------------|----------|-----------------|-----------|------------|
|          |            |               | Dielectric Strength (KV) |           |           | Dissipation Factor |          |                 |           |            |
|          |            |               | AC                       | Impulse   | Breakdown | Positive           | Negative | (tan $\delta$ ) | at 25° C. | at 100° C. |
| Example  | (Volume %) | Particle Type | Gauss                    | Breakdown |           |                    |          | (% of Total)    |           | Stability  |
| 1H       | 0.6        | magnetic      | 30                       | 54        | 120       | 125                | 1.5      | 8               | 1         | stable     |
| 1I       | 0.6        | non-magnetic  | 0                        | 55        | 110       | 120                | 0.4      | 2.5             | 0.1       | stable     |
| 1J       | 0.1        | magnetic      | 5                        | 54        | 120       | 120                | 1.2      | 4.5             | 0.4       | stable     |
| 1K       | 0.1        | non-magnetic  | 0                        | 55        | 125       | 120                | 0.06     | 0.3             | 0         | stable     |
| 1L       | 0.01       | magnetic      | 0.5                      | 55        | 115       | 125                | 0.1      | 0.4             | 0.1       | stable     |
| 1M       | 0.01       | non-magnetic  | 0                        | 55        | 115       | 125                | 0.009    | 0.05            | 0         | stable     |

Note:

Ms is saturation magnetization

Inspection of the data in Table 1 reveals that colloids within the scope of the present invention (as exemplified, for example, by Examples 1E and 1G through 1M), which may comprise a dispersed phase concentration of up to about 2% by volume and a saturation magnetization (Ms) of less than about 50 Gauss, exhibit significantly improved dielectric

20  
tion fluids for a 50 KVA transformer operating at a temperature of about 70° C. A cooling fluid containing oil only (Example 2A) was run as a control. Temperature readings were taken at different locations (top, middle, bottom) around the transformer windings and cooling fins. The resulting data is tabulated below.

TABLE 2

| Ms | Zone Where Temperature Rise Was Measured |         |          |        |        |              |      |        |        |
|----|------------------------------------------|---------|----------|--------|--------|--------------|------|--------|--------|
|    | Example                                  | (Gauss) | Windings |        |        | Cooling Fins |      |        |        |
|    |                                          |         | Top      | Middle | Bottom | Average      | Top  | Middle | Bottom |
| 2A | 0                                        | 71.3    | 67.6     | 53.6   | 64.2   | 56.1         | 54.2 | 39.5   | 49.9   |
| 2B | 200                                      | 75.1    | 65.5     | 56     | 65.5   | 48.3         | 53.5 | 38     | 46.6   |
| 2C | 50                                       | 74.7    | 66.3     | 54.7   | 65.2   | 51.2         | 52.4 | 38.5   | 47.4   |
| 2D | 30                                       | 63.5    | 64       | 51.5   | 59.7   | 54.2         | 53   | 39     | 48.7   |
| 2E | 10                                       | 66.2    | 65.1     | 52.7   | 61.3   | 55.5         | 53.3 | 39.1   | 49.3   |
| 2F | 5                                        | 67      | 65.5     | 53     | 61.8   | 56           | 54   | 39.2   | 49.7   |
| 2G | 1                                        | 71      | 67.5     | 53.5   | 64     | 56           | 54   | 39.6   | 49.9   |

Notes:

1. Transformer was loaded at 110%: Voltage = 200 V; Current = 275 A.

strengths as compared to colloidal fluids of the prior art which include dispersed phase concentrations of greater than about 2% by volume and an Ms of about 50 Gauss or greater (see Examples 1B through 1D and 1F) and pure oil (see Example 1A). Specifically, colloids within the scope of the present invention possess increased positive values for the impulse breakdown strength as compared to colloids of the prior art. The data reveals also that colloids within the scope of the present invention possess improved dissipation factors at both ambient temperature (25° C.) and at elevated temperature (100° C.).

### Example 2

This example includes a description of experiments which were conducted to evaluate and compare the cooling performance of colloidal fluids within the scope of the present invention to the cooling performance of colloidal fluids of the prior art.

Colloidal fluids having saturation magnetization values of 1, 5, 10, 30, 50 and 200 Gauss were prepared by making various dilutions in oil of a colloid of magnetite ( $\text{FeO}\cdot\text{Fe}_2\text{O}_3$ ). These colloidal fluids were utilized as insula-

45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790

## 13

heated colloidal fluid 12 and vector  $F_C$  which indicates the downwards component of the Archimedes force acting on cooled portions of the colloidal fluid 12. Vector  $F_A$  is substantially identical with the colloidal fluids of the present invention as with conventional oils of the prior art which may be used as the carrier oil in the present colloidal fluids. Vector  $F_M$  is the force due to the magnetic interaction of the colloidal fluid 12 with the magnetic field created by windings 16.

The Descartes axes 18 shows the magnetic field density of across the windings 16.  $B_O$  is the magnetic induction between the windings, and  $B$  is the magnetic induction inside the magnetic core. This magnetic field gradient results in a pressure drop across the windings 16 and results in magnetohydronamic convection.

## Example 3

Experiments were conducted to evaluate the effect of particle size on the electrical resistivity and dielectric strength of colloidal cooling fluids within the scope of the present invention. The results of these experiments are tabulated in Table 3 below.

TABLE 3

| Magnetization Saturation<br>(Gauss) | Resistivity<br>( $10^{10}$ Ohm · cm) For<br>Varying Particle Size (nm) |    |     | Loss Increase (% of<br>total) For Varying<br>Particle Size (nm) |     |     |
|-------------------------------------|------------------------------------------------------------------------|----|-----|-----------------------------------------------------------------|-----|-----|
|                                     | <7                                                                     | 9  | >10 | <7                                                              | 9   | >10 |
| 30                                  | 1.5                                                                    | 5  | 12  | 6                                                               | 1.0 | 0.7 |
| 10                                  | 4                                                                      | 12 | 30  | 2.8                                                             | 0.5 | 0.3 |
| 5                                   | 7                                                                      | 20 | 50  | 1.5                                                             | 0.2 | 0.1 |

Inspection of the data set forth in Table 3 indicates that increasing the average particle size from less than about 7 nm to greater than about 10 nm results in about a ten-fold increase in electric Resistivity as well as about a ten-fold decrease in power loss associated with the conductive component of dielectric loss.

The disclosures of each patent, patent application and publication cited or described in this document are hereby incorporated by reference, in their entirety.

Various modifications of the invention, in addition to those described herein, will be apparent to those skilled in the art from the foregoing description. Such modifications are also intended to fall within the scope of the appended claims.

What is claimed is:

1. A stable colloidal fluid comprising:
  - (a) about 99.99 to about 99.5% by volume of a carrier liquid; and
  - (b) from about 0.01 to about 0.5% by volume of non-metallic particles, wherein the colloidal fluid has a saturation magnetization of from about 1 to about 20 Gauss, and wherein said particles are magnetic particles.
2. A colloidal fluid according to claim 1 which has an electrical resistivity of at least about  $10^9$  ohm·cm.
3. A colloidal fluid according to claim 2 which has an electrical resistivity of from about  $10^9$  ohm·cm to about  $10^{13}$  ohm·cm.
4. A colloidal fluid according to claim 3 which has an electrical resistivity of greater than about  $10^{13}$  ohm·cm.

## 14

5. A colloidal fluid according to claim 1 wherein said carrier liquid comprises an oil.

6. A colloidal fluid according to claim 1 wherein said particles comprise inorganic particles.

7. A colloidal fluid according to claim 6 wherein said particles are selected from the group consisting of metal oxides.

8. A colloidal fluid according to claim 7 wherein said particles comprise oxides of metals selected from the group consisting of iron, zinc, manganese, titanium, copper, nickel, chromium, and combinations thereof.

9. A colloidal fluid according to claim 1 which further comprises a stabilizing material.

10. A colloidal fluid according to claim 9 wherein said stabilizing material comprises a surfactant.

11. A colloidal fluid according to claim 1 which has a saturation magnetization of from about 5 to about 20 Gauss.

12. A colloidal fluid according to claim 1 wherein the size of said particles ranges from about 1 to about 100 nm.

13. A colloidal fluid according to claim 12 wherein said particles have an average particle size of from about 5 to about 20 nm.

14. A colloidal fluid according to claim 13 wherein said particles have an average particle size of from about 7 to about 20 nm.

15. A colloidal fluid according to claim 1 which provides an increase in the positive value of impulse breakdown voltage of at least about 10%.

16. A method for preparing a stable colloidal fluid having a saturation magnetization of from about 1 to about 20 Gauss, wherein the method comprises:

(a) providing about 99.99 to about 99.5% by volume of a carrier liquid; and

(b) combining from about 0.01 to about 0.5% by volume of non-metallic particles with said carrier liquid, wherein said particles are magnetic particles.

17. A method according to claim 16 wherein said carrier liquid comprises an oil.

18. A method according to claims 16 wherein said particles comprise inorganic particles.

19. A method according to claim 16 wherein said colloidal fluid has an electrical resistivity of greater than about  $10^9$  ohm·cm.

20. An electromagnetic device comprising:

(a) means for producing an electromagnetic field and heat; and

(b) a stable, colloidal insulating fluid which is in contact with said device and which comprises:

(i) a carrier liquid; and

(ii) non-metallic particles;

55 wherein the colloidal insulating fluid has a saturation magnetization of from about 1 to about 20 Gauss.

21. An electromagnetic device according to claim 20 which is a power transformer.

22. A method of insulating and cooling an electromagnetic device which produces an external magnetic field and heat, wherein the method comprises contacting the device with a stable, colloidal insulating fluid comprising:

(a) a carrier liquid; and

(b) non-metallic particles;

65 wherein the colloidal insulating fluid has a saturation magnetization of from about 1 to about 20 Gauss.

**15**

- 23.** A stable colloidal fluid comprising:
- (a) about 99.99 to about 99.5% by volume of a carrier liquid; and
  - (b) from about 0.01 to about 0.5% by volume of non-metallic particles, wherein the colloidal fluid has a saturation magnetization of from about 0 to about 25 Gauss, and wherein said particles are magnetic particles.

**16**

- 24.** A colloidal fluid according to claim **23** which has a saturation magnetization of from about 0.5 to less than about 5 Gauss.

- 25.** A colloidal fluid according to claim **23** which has a saturation magnetization of from about 10 to about 25 Gauss.

\* \* \* \* \*